# EUROPEAN PATENT SPECIFICATION

(11) **EP 0 709 477 B1**
(45) Date of publication and mention of the grant of the patent: **27.05.1998**
(21) Application number: 95114242.1
(22) Date of filing: 11.09.1995
(51) Int. Cl.: C22C 19/05

(54) **Heat-resistant nickel-based alloy excellent in weldability**
Schweissbare und hitzebeständige Legierung auf Nickelbasis
Alliage réfractaire et soudable à base de nickel

(30) Priority: 31.10.1994 JP 267111/94
(43) Date of publication of application: 01.05.1996
(73) Proprietor: MITSUBISHI STEEL MFG. CO., LTD., Tokyo (JP); MITSUBISHI JUKOGYO KABUSHIKI KAISHA, Tokyo 100 (JP)
(72) Inventor: Tamura, Itaru c/o Mitsubishi Steel MFG. CO. LTD.,, Tokyo (JP); Tokoro, Kazunori c/o Mitsubishi Steel MFG. CO.LTD, Tokyo (JP); Kawabata, Takashi c/o Mitsubishi Steel MFG. CO. LT, Utsunomiya-shi Tochigi (JP); Kokubun, Tsuyoki c/o Mitsubishi Steel MFG. CO. LT, Utsunomiya-shi Tochigi (JP); Mochizuki, Toshio c/o Mitsubishi Steel MFG. CO., Utsunomiya-shi Tochigi (JP); Sakashita, Shuichi c/o Mitsubishi Steel MFG. CO., Utsunomiya-shi Tochigi (JP); Kawai, Hisataka c/o Mitsubishi Jukogyo K.K., 2-chome, Takasago-shi Hyogo (JP); Okada, Ikuo c/o Mitsubishi Jukogyo K.K., 2-chome, Takasago-shi Hyogo (JP); Tsuji, Ichiro c/o Mitsubishi Jukogyo K.K., 2-chome, Takasago-shi Hyogo (JP); Takahashi,Kouji c/o Mitsubishi Jukogyo K.K., 2-chome, Takasago-shi Hyogo (JP); Torigoe, Taiji c/o Mitsubishi Jukogyo K.K., 2-chome, Takasago-shi Hyogo (JP)
(74) Representative: Sandmair, Kurt, Dr. Dr.

(56) References cited:
- EP-A- 0 302 302
- EP-A- 0 361 524
- EP-A- 0 561 179
- GB-A- 1 367 661
- US-A- 4 039 330

## Description

### 1. Field of the Invention

The present invention relates to a heat-resistant nickel-based alloy that can be used as a material for forming the stationary turbine vane of a gas turbine and other parts to be exposed to high temperatures.

### 2. Description of the Prior Art

Heat-resistant alloys heretofore used as materials for parts to be exposed to high temperatures, such as the stationary turbine vane of a gas turbine, include an Ni-based alloy which enjoys the effects of both strengthening through precipitation of an intermetallic compound Ni₃(Al,Ti), i.e., a γ' phase, and strengthening through solid solution with Mo, W, etc., and a Co-based alloy strengthened through precipitation of a carbide.

In the Ni-based alloy, an increase in the amount of precipitation of the γ' phase generally tends to lower the weldability of the alloy, though it improves the high-temperature strength of the alloy. For example, this is clear from the fact that an alloy increased in the amount of precipitation of the γ' phase to improve the high-temperature strength thereof (Japanese Patent Publication No. 6,968/1979) is very poor in weldability, while an alloy decreased in the amount of precipitation of the γ' phase to improve the weldability thereof (Japanese Patent Laid-Open No. 104,738/1989) is very low in high-temperature strength. On the other hand, the Co-based alloy, though generally good in weldability, is low in high-temperature strength, and no remarkable improvement can be expected.

As is apparent from the foregoing, since the high-temperature strength of the Co-based alloy is limited, the Ni-based alloy must be improved in weldability without detriment to the high-temperature strength thereof.

### SUMMARY OF THE INVENTION

In order to improve the weldability of the Ni-based alloy without detriment to the high-temperature strength thereof, the contents of γ' phase-forming elements such as Al and Ti should not be lowered, but the contents of other elements such as W, C, and Zr must be adjusted for the desired purpose of obtaining an alloy which can be used to produce, for example, welded structures to be used at high temperatures, such as the stationary vane of a gas turbine and apparatuses having a welded structure. The performance of such an alloy is characterized by a creep rupture life of at least 110 hours as measured under 20 kgf/mm² at 900°C, and a maximum crack length of at most 0.8 mm, as measured using 5x60x100 mm test pieces TIG-welded to each other under welding conditions involving a welding current of 100 A, a welding voltage of 12 V and a welding speed of 1.67 mm/sec, according to a varestraint test wherein the added strain (total strain) is 0.25% or 0.77%.

As a result of intensive investigations, the inventors of the present invention have found out that an alloy having an excellent high-temperature strength and a good weldability can be obtained by increasing the high-temperature strength through the addition of Cr and Co within such respective ranges of contents as not to form deleterious phases such as a σ phase and a µ phase and further addition of γ' phase-forming elements such as Al, Ti, Nb and Ta as well as solid solution strengthening elements, such as W and Mo, while at the same time improving the weldability through the addition of suitable amounts of C, Zr and B liable to segregate in grain boundaries, as corresponds to an alloy composition which will be described later; and that a Ni-based alloy usable as a material for parts to be exposed to high temperatures and used in a low-grade fuel such as heavy oil, i.e., having excellent oxidation resistance and corrosion resistance as well, can be prepared. The present invention has been completed based on these findings.

Specifically, in accordance with the present invention, there are provided:
(1) a heat-resistant nickel-based alloy comprising, in terms of wt. %, 0.05 to 0.25% of C, 18 to 25% of Cr, 15 to 25% of Co, up to 3.5% of Mo and more than 5 to 10% of W with the content of one or both of Mo and W being more than 5 to 10% in terms of W + 1/2MO, 1.0 to 5.0% of Ti, 1.0 to 4.0% of Al, 0.5 to 4.5% of Ta, 0.2 to 3.0% of Nb, 0.005 to 0.10% of Zr, 0.001 to 0.01% of B, and the balance being Ni and unavoidable impurity elements, wherein the (Al + Ti) content and the (W + 1/2Mo) content are within the range surrounded by the line connecting the point A (Al + Ti: 3%, W + 1/2Mo: 10%), the point B (Al + Ti: 5%, W + 1/2Mo: 7.5%), the point C (Al + Ti: 5%, W + 1/2Mo: 5%), the point D (Al + Ti: 7%, W + 1/2Mo: 5%), and the point E (Al + Ti: 7%, W + 1/2Mo: 10%) in this sequence in Fig. 1; and
(2) a heat-resistant nickel-based alloy comprising, in terms of wt. %, 0.05 to 0.25% of C, 10 to less than 20% of Cr, 15 to 25% of Co, up to 3.5% of Mo and 0.5 to 10% of W, with the content of one or both of Mo and W being 0.5 to 10% in terms of W + 1/2Mo, 1.0 to 5.0% of Ti, 1.0 to 4.0% of Al, 0.5 to 4.5% of Ta, 0.2 to 3.0% of Nb, 0.005 to 0.10% of Zr, 0.001 to 0.01% of B, and the balance being Ni and unavoidable impurity elements, wherein the (Al + Ti) content and the (W + 1/2Mo) content are within the range surrounded by the line connecting the point A (Al + Ti: 3%, W + 1/2Mo: 10%), the point B (Al + Ti: 5%, W + 1/2Mo: 7.5 %), the point C (Al + Ti: 5%, W + 1/2Mo: 5%), the point F (Al + Ti: 4 %, W + 1/2Mo: 5%), the point G (Al + Ti: 4%, W + 1/2Mo: 0.5%), the point H (Al + Ti: 7%, W + 1/2Mo: 0.5%), and the point E (Al + Ti: 7%, W + 1/2Mo: 10%) in this sequence in Fig. 1.

### BRIEF DESCRIPTION OF THE DRAWINGS

Fig. 1 is a diagram showing the scope of the alloy of the present invention and the test results with respect to creep rupture life.

Fig. 2 is a diagram showing a comparison of alloys tested for creep rupture strength.

Fig. 3 is a diagram showing the relationship between the maximum varestraint crack length and the creep rupture life.

Fig. 4 is a perspective view of the stationary vane of a gas turbine produced using the alloy of the present invention and subjected to a weldability test.

Fig. 5 is an illustration of the welded portion in the weldability test.

Figs. 6A and 6B are illustrations of the essentials of the varestraint test carried out for the evaluation of weldabilities of alloys according to the present invention and comparative alloys.

### DETAILED DESCRIPTION OF THE PREFERRED EMBODIMENTS

The functions of elements in the alloy composition of the heat-resistant Ni-based alloy of the present invention will now be described together with the reasons for specifying the contents (by weight) of the elements added thereto.

C forms a carbide which precipitates particularly in crystal grain boundaries and in dendrite boundaries to strengthen the grain boundaries and the dendrite boundaries. When the C content is lower than 0.05%, the strengthening effect thereof is negligible. When it exceeds 0.25%, the ductility and creep strength of the alloy are lowered. It is especially preferably in the range of 0.09 to 0.23%.

The Cr content is specified to be 18 to 25% in the foregoing nickel-based nickel alloy (1) of the first type and 10 to less than 20% in the nickel-based nickel alloy (2) of the second type. Cr is an element capable of imparting an oxidation resistance and a corrosion resistance at high temperatures to the alloy. When the Cr content is lower than the above-specified lower limits, the effect thereof is poor. When it exceeds the above-specified upper limits, it involves a fear of forming the a phase when the alloy is used at a high temperature for a long period of time. Additionally stated, the nickel-based nickel alloy (1) ) is provided having particular regard to the corrosion resistance and oxidation resistance thereof, while the nickel-based nickel alloy (2) is provided having particular regard to the high-temperature strength thereof.

Co has a function of increasing the limit of solid solution (solid solution limit) of γ' phase-forming elements such as Ti and Al into the matrix at a high temperature. With the Al and Ti contents of the alloy according to the present invention, a Co content'of at least 15.0% must be adopted. On the other hand, the Co content is specified to be at most 25.0% in order to avoid a fear of forming the σ phase.

Ti is an element required for precipitation of the γ' phase to increase the high-temperature strength of the alloy. When the Ti content is lower than 1.0%, the desired strength cannot be secured. On the other hand, it is specified to be at most 5.0% because too much addition of Ti spoils the ductility and weldability of the alloy.

Al forms the γ' phase like Ti to increase the high-temperature strength of the alloy while contributing to imparting to the alloy an oxidation resistance and a corrosion resistance at high temperatures. The Al content must be at least 1.0%, while it is specified to be atmost 4.0% because too much addition of Al spoils the ductility and weldability of the alloy. The (Al + Ti) content is especially preferably in the range of 3.0 to 7.0%.

W and Mo have a function of solid solution strengthening and,weak precipitation strengthening to contribute to imparting a high-temperature strength to the alloy. In order to secure the foregoing effect, the (W + 1/2Mo) content must be at least 0.5%. Since too much addition of these elements spoils the ductility of the alloy, the W content, the Mo content, and the (W + 1/2Mo) content are specified to be at most 10%, at most 3.5%, and at most 10%, respectively.

Ta and Nb contribute to an improvement in high-temperature strength through solid solution strengthening and γ' phase precipitation strengthening. This effect is exhibited when the Ta content is at least 0.5% and when the Nb content is at least 0.2%. On the other hand, since too much addition of these elements lowers the ductility of the alloy, the Ta content and the Nb content are specified to be at most 4.5% and at most 3.0%, respectively. The Ta content and the Nb content are especially preferably in the range of 1.0 to 4.2% and in the range of 0.5 to 1.5%, respectively.

Zr exhibits the effect of increasing the bonding strength in crystal grain boundaries to strengthen the grain boundaries. When the Zr content is lower than 0.005%, no improvement in creep strength can be observed. On the other hand, when it exceeds 0.10%, the weldability of the alloy is unfavorably lowered. Thus, it must be in the range of 0.005 to 0.10%, and is especially preferably in the range of 0.01 to 0.10%.

B increases the bonding strength in crystal grain boundaries like Zr to strengthen the grain boundaries. When the B content is lower than 0.001%, no improvement in creep strength can be observed. On the other hand, when it exceeds 0.01%, the weldability of the alloy is unfavorably lowered. Thus, the B content is specified to be in the range of 0.001 to 0.01%.

The reasons why limitations are made within the ranges surrounded by the lines in Fig. 1 are as follows. Al and Ti precipitate the γ' phase, i.e., Ni₃(Al, Ti), as a factor in strengthening the Ni-based alloy to increase the high-temperature strength thereof. Since too much addition of these elements lowers the weldability and ductility of the alloy, however, the (Al + Ti) content is specified to be at most 7%. When it is too low, the effect of increasing the high-temperature strength of the alloy is decreased. Thus, it is specified to be at least 3% as shown in the same figure. Additionally stated, since the Cr content also exerts an influence on the high-temperature strength of the alloy, the lower limit of the (Al + Ti) content is specified, with taking also into account the Cr content, to be at least 4%, as shown in the same figure. W and Mo have a function of solid solution strengthening and carbide precipitation strengthening to exhibit the effect of increasing the high-temperature strength of the alloy. In order to secure this effect, the (W + 1/2Mo) content must be at least 0.5%. On the other hand, since too much addition of these elements fosters precipitation of deleterious phases such as the a phase to lower the ductility and strength of the alloy, the upper limit of the (W + 1/2Mo) content is specified to be 10%.

The following specific Examples will illustrate the present invention in more detail.

### Example 1

Table 1 shows the chemical compositions (by wt.%) of representative alloys invented for the stationary vane of a gas turbine. On the other hand, Table 2 shows the chemical compositions of comparative alloys as conventional alloys. Each composition was melted in a high-frequency vacuum melting furnace to prepare 20 kg of an ingot. This sample was precision-cast as the master ingot according to a lost wax process, and then heat-treated at 1,160°C for 4 hours, at 1,000°C for 6 hours, and at 800°C for 4 hours. Thereafter, it was machined into creep rupture test pieces of 6.25 mm φ x 25 mm in parallel portion size, 5x60x100 mm varestraint test pieces, etc. Alloys Nos. 1 to 18 in Table 1 are alloys according to the present invention, while Alloys Nos. X, Y, Z, and 19 to 36 are comparative alloys. Additionally stated, the Alloys Nos. X and Y are examples of the aforementioned alloy of Japanese Patent Publication No. 6,968/1979, while the Alloy No. Z is an example of the aforementioned alloy of Japanese Patent Laid-Open No. 104,738/1989.

Fig. 1 shows the relationship between the (Al + Ti) content and the (W + 1/2Mo) content for every sample as well as the creep rupture life under 20 kgf/mm² at 900°C in ( ) accompanying every sample No. Additionally stated, in Fig. 1, the alloys according to the present invention were indicated by the open symbol (o), while the comparative alloys are indicated by the solid symbol (●).

Alloys of the present invention with high (Al + Ti) and (W + 1/2Mo) contents which are in the range surrounded by the line connecting points A, B, C, D, and E (1, 4, 11, 12, 13, 14, 15, and 16) all exhibit a high strength, and Alloy No. 11 in particular exhibits an especially high strength. Alloys of the present invention with a low Cr content and with (Al + Ti) and (W + 1/2Mo) contents which are in the range surrounded by the line connecting points F, G, H, and D (2, 3, 5, 6, 7, 8, 9, 10, 17, and 18) exhibit an especially high strength.

Fig. 2 shows a comparison of Alloys Nos. 9 and 11 of the present invention in Table 1 with the Comparative Alloys Nos. Y, Z, and 20 in Table 2 with respect to creep rupture strength under 20 kgf/mm² at 900°C and under 10 kgf/mm² at 980°C. The abscissa represents the Larson-Miller parameter: P = Tₖx:(20 + log t)x10⁻³ [Tₖ : test temperature (°K), t: rupture life (hr)]. The test results at 900°C and 980°C correspond to the points of 20 kgf/mm² and 10 kgf/mm², respectively, in terms of stress represented by the ordinate. It is demonstrated that the higher the parameter P in the abscissa, the higher the strength. Alloys Nos. 9 and 11 of the present invention are higher in Larson-Miller parameter under the same test stress than the Comparative Alloys Nos. Y, Z, and 20. This is the effect of increasing the (Al + Ti) content and the (W + 1/2Mo) content while decreasing the Cr content (No.11). On the other hand, Comparative Alloy No. Y which was slightly higher in (Al + Ti) content than the Alloy No. 9 and high also in Cr content, Comparative Alloy No. 20 which was low in (Al + Ti) content but high in (W + 1/2Mo) content, Comparative Alloy No. Z which was low in both of (Al + Ti) content and (W + 1/2Mo) content, etc. are lower in Larson-Miller parameter under the same test stress than the alloys of the present invention.

The weldability was evaluated according to a varestraint test, as shown in Figs. 6A and 6B. In the figures, reference numerals are as follows: 12: varestraint test piece (before application of flexural stress), 13: yoke, 14: bead, 15: welding torch, 16: varestraint test piece (after application of flexural stress), and 17: bending block.

Specifically, test pieces were TIG-welded to each other under welding conditions involving a welding current of 100 A, a welding voltage of 12 V, and a welding speed of 1.67 mm/sec, and then loaded with a total strain of 0.25% or 0.77%. The resulting maximum crack length as a yardstick of the zone turned brittle when welded was measured. Fig. 3 shows the relationship between the maximum crack length and the creep rupture life (900°C x 20 kgf/mm²). The ordinate in the same figure demonstrates that the smaller the maximum crack length, the better the weldability. Accordingly, as the point is located at the furtherest right side and at the lower side, the alloy is higher in high-temperature strength and better in weldability, respectively. The Alloys Nos. 3, 7, 9, 10, 11, 12, and 15 with a Zr content of at most 0.1% and a B content of at most 0.01 according to the present invention are all small in maximum crack length in the varestraint test. Alloys Nos. 9, 11, and 12 in particular showed a maximum crack length of at most 0.3 mm as the target and a creep rupture life of at least 185 hours, and hence have excellent properties. On the other hand, Comparative Alloys Nos. X, Y, 25, 27, 28, 33, and 35 all showed a maximum crack length in the varestraint test of at least 0.8 mm to miss the target, though they showed a creep rupture life of at least 110 hours. As is apparent from the foregoing results, a good weldability and a high creep strength can be secured either if the relationship between the (Al + Ti) content and the (W + 1/2Mo) content are specified to be in the range A-B-C-D-E even though the Zr content and the B content are lowered, or if the relationship between the (Al + Ti) content and the (W + 1/2Mo) content are specified to be in the range A-B-C-F-G-H-E with a decrease in Cr content.

### Example 2

Alloy No. 11 of Example 1, as shown in Table 1, was used to produce the stationary vane of a gas turbine as shown in Fig. 4 according to the lost wax precision-casting process. The resulting product was subjected to a solution heat treatment at 1,160°C for 4 hours, and then subjected to a weldability test. The stationary vane had a profile portion width of about 200 mm and a height of about 200 mm, and was a cast article having a hollow structure provided with an internal air path for cooling the same. As shown in Fig. 4, build-up welding, or padding, was carried out in ventral places 1, 2, 3, and 4 of a vane portion, places 5 and 6 of the leading edge, and a place 7 of the trailing edge. Reference numeral 9 represents an outer shroud. As shown in Fig. 5, the shroud portion 8 (Alloy No. 11 of the present invention) of the inner shroud 8 was welded with a cover plate 10 (Hastelloy X alloy) with a fillet welding of Hastelloy W alloy 11 according to the TIG welding method. After the welding, a visual inspection, a fluorescence penetrant inspection, an observation of the microstructure of the cross section at the position as shown in Fig. 5, etc. were carried out and no cracks were found in any place. Additionally stated, substantially the same stationary vane of a gas turbine as described above was produced using Comparative Alloy No. Y (Japanese Patent Publication No. 6,968/1979), and subjected to a weldability test. As a result, many cracks were found by a fluorescence penetrant inspection, while cracks of about 1 mm in length were found by an observation of the microstructure of the cross section.

As described hereinbefore, according to the present invention, a heat-resistant Ni-based alloy can be obtained, which has a higher high-temperature strength and a better weldability than conventional heat-resistant Ni-based alloys. This heat-resistant Ni-based alloy is especially suitable as a material for the stationary vane of a gas turbine required to be reliable in keeping with an increase in the service temperature of the gas turbine.

## Claims

1. A heat-resistant nickel-based alloy excellent in weldability, said nickel-based alloy comprising, in terms of wt. %, 0.05 to 0.25% of C, 18 to 25% of Cr, 15 to 25% of Co, up to 3.5% of Mo and 5 to 10% of W with the proviso to exclude an amount of W of 5 % with the content of one or both of Mo and W being 5 to 10% in terms of W + 1/2Mo excluding an amount of 5 % of W + 1/2Mo, 1.0 to 5.0% of Ti, 1.0 to 4.0% of Al, 0.5 to 4.5% of Ta, 0.2 to 3.0% of Nb, 0.005 to 0.10% of Zr, 0.001 to 0.01% of B, and the balance of Ni and unavoidable impurity elements, wherein the (Al + Ti) content and the (W + 1/2Mo) content are within the range surrounded by the line connecting the point A (Al + Ti: 3%, W + 1/2Mo: 10%), the point B (Al + Ti: 5%, W + 1/2Mo: 7.5%), the point C (Al + Ti: 5%, W + 1/2Mo: 5%), the point D (Al + Ti: 7%, W + 1/2Mo: 5%), and the point E (Al + Ti: 7%, W + 1/2Mo: 10%) in this sequence in Fig. 1.

2. A heat-resistant nickel-based alloy excellent in weldability, said nickel-based alloy comprising, in terms of wt. %, 0.05 to 0.25% of C, 10 to 20% of Cr with the proviso that the amount of Cr of 20 % is excluded, 15 to 25% of Co, up to 3.5% of Mo and 0.5 to 10% of W with the content of one or both of Mo and W being 0.5 to 10% in terms of W + 1/2Mo, 1.0 to 5.0% of Ti, 1.0 to 4.0% of Al, 0.5 to 4.5% of Ta, 0.2 to 3.0% of Nb, 0.005 to 0.10% of Zr, 0.001 to 0.01% of B, and the balance of Ni and unavoidable impurity elements, wherein the (Al + Ti) content and the (W + 1/2Mo) content are within the range surrounded by the line connecting the point A (Al + Ti: 3%, W + 1/2Mo: 10%), the point B (Al + Ti: 5%, W + 1/2Mo: 7.5%), the point C (Al + Ti: 5%, W + 1/2Mo: 5%), the point F (Al + Ti: 4%, W + 1/2Mo: 5%), the point G (Al + Ti: 4%, W + 1/2Mo: 0.5%), the point H (Al + Ti: 7%, W + 1/2Mo: 0.5%), and the point E (Al + Ti: 7%, W + 1/2Mo: 10%) in this sequence in Fig. 1.

## Patentansprüche

1. Wärmebeständige Legierung auf Nickelbasis, die sich sehr gut schweißen läßt und in Gew.-% 0,05 bis 0,25 % C, 18 bis 25 % Cr, 15 bis 25 % Co, bis zu 3,5 % Mo und 5 bis 10 % W, mit der Maßgabe, daß eine W-Menge von 5 % ausgeschlossen ist, wobei der Gehalt an Mo und/oder W bezogen auf W + ½ Mo 5 bis 10 % beträgt und eine Menge von 5 % W + ½ Mo ausgeschlossen ist, 1,0 bis 5,0 % Ti, 1,0 bis 4,0 % Al, 0,5 bis 4,5 % Ta, 0,2 bis 3,0 % Nb, 0,005 bis 0,10 % Zr, 0,001 bis 0,01 % B enthält und der Rest aus Ni und unvermeidlichen Verunreinigungselementen besteht, wobei der Gehalt an (Al + Ti) und der Gehalt an (W + ½ Mo) in dem Bereich liegt, der durch die den Punkt A (Al + Ti: 3 %, W + ½ Mo: 10 %), den Punkt B (Al + Ti: 5 %, W + ½ Mo: 7,5 %), den Punkt C (Al + Ti: 5 %, W + ½ Mo: 5 %), den Punkt D (Al + Ti: 7 %, W + ½ Mo: 5 %) und den Punkt E (Al + Ti: 7 %, W + ½ Mo: 10 %) verbindenden Linie in dieser Sequenz in Fig. 1 umgeben ist.

2. Wärmebeständige Legierung auf Nickelbasis, die sich sehr gut schweißen läßt und in Gew.-% 0,05 bis 0,25 % C, 10 bis 20 % Cr, mit der Maßgabe, daß eine Cr-Menge von 20 % ausgeschlossen ist, 15 bis 25 % Co, bis zu 3,5 % Mo und 0,5 bis 10 % W, wobei der Gehalt an Mo und/oder W bezogen auf W + ½ Mo 0,5 bis 10 % beträgt, 1,0 bis 5,0 % Ti, 1,0 bis 4,0 % Al, 0,5 bis 4,5 % Ta, 0,2 bis 3,0 % Nb, 0,005 bis 0,10 % Zr, 0,001 bis 0,01 % B enthält und der Rest aus Ni und unvermeidlichen Verunreinigungselementen besteht, wobei der Gehalt an (Al + Ti) und der Gehalt an (W + ½ Mo) in dem Bereich liegt, der durch die den Punkt A (Al + Ti: 3 %, W + ½ Mo: 10 %), den Punkt B (Al + Ti: 5 %, W + ½ Mo: 7,5 %), den Punkt C (Al + Ti: 5 %, W +½ Mo: 5 %), den Punkt F (Al + Ti: 4 %, W + ½ Mo: 5 %), den Punkt G (Al + Ti: 4 %, W + ½ Mo: 0,5 %), den Punkt H (Al + Ti: 7 %, W + ½ Mo: 0,5 %) und den Punkt E (Al + Ti: 7 %, W + ½ Mo: 10 %) verbindenden Linie in dieser Sequenz in Fig. 1 umgeben ist.

## Revendications

1. Alliage à base de nickel résistant à la chaleur ayant une excellente aptitude au soudage, ledit alliage à base de nickel comprenant, en pourcentage en poids, entre 0,05 et 0,25% de C, entre 18 et 25% de Cr, entre 15 et 25% de Co, jusqu'à 3,5% de Mo et entre 5 et 10% de W, à la condition que la quantité de W de 5% soit exclue, la teneur en l'un ou les deux parmi Mo et W étant comprise entre 5 et 10% en termes de W + 1/2Mo, en excluant une quantité de 5% de W + 1/2Mo, entre 1,0 et 5,0% de Ti, entre 1,0 et 4,0% de Al, entre 0,5 et 4,5% de Ta, entre 0,2 et 3,0% de Nb, entre 0,005 et 0,10% de Zr, entre 0,001 et 0,01% de B, le reste étant du Ni et des éléments d'impuretés inévitables, dans lequel la teneur en (Al + Ti) et la teneur en (W + 1/2Mo) sont comprises dans la zone entourée par la ligne connectant le point A (Al + Ti : 3%, W + 1/2Mo : 10%), le point B (Al + Ti : 5%, W + 1/2Mo : 7,5%), le point C (Al + Ti : 5%, W + 1/2Mo : 5%), le point D (Al + Ti : 7%, W + 1/2Mo : 5%), et le point E (Al + Ti : 7%, W + 1/2Mo : 10%), dans cet ordre, en figure 1.

2. Alliage à base de nickel résistant à la chaleur ayant une excellente aptitude au soudage, ledit alliage à base de nickel comprenant, en pourcentage en poids, entre 0,05 et 0,25% de C, entre 10 et 20% de Cr, à la condition que la quantité de Cr de 20% soit exclue, entre 15 et 25% de Co, jusqu'à 3,5% de Mo et entre 0,5 et 10% de W, la teneur en l'un ou les deux parmi Mo et W étant comprise entre 0,5 et 10% en termes de W + 1/2Mo, entre 1,0 et 5,0% de Ti, entre 1,0 et 4,0% de Al, entre 0,5 et 4,5% de Ta, entre 0,2 et 3,0% de Nb, entre 0,005 et 0,10% de Zr, entre 0,001 et 0,01% de B, le reste étant du Ni et des éléments d'impuretés inévitables, dans lequel la teneur en (Al + Ti) et la teneur en (W + 1/2Mo) sont comprises dans la zone entourée par la ligne connectant le point A (Al + Ti : 3%, W + 1/2Mo : 10%), le point B (Al + Ti : 5%, W + 1/2Mo : 7,5%), le point C (Al + Ti : 5%, W + 1/2Mo : 5%), le point F (Al + Ti : 4%, W + 1/2Mo : 5%), le point G (Al + Ti : 4%, W + 1/2Mo : 0,5%), le point H (Al + Ti : 7%, W + 1/2Mo : 0,5%), et le point E (Al + Ti : 7%, W + 1/2Mo : 10%), dans cet ordre, en figure 1.
